

1

3,309,315  
SULPHURIZED CUTTING OIL AND PROCESS  
OF MAKING SAME

John Hanna J. Tarazi and Herbert D. Ivey, Jr., Pasadena, Calif., assignors to Lubrication Company of America, Los Angeles, Calif.

No Drawing. Filed Aug. 14, 1963, Ser. No. 301,986  
21 Claims. (Cl. 252—42.4)

Cutting oils used in the machining of steel and the like, require an active sulfur compound in the oil; that is, a compound which at a temperature lower than the welding temperature of steel forms iron sulfide on the tool and work surface so as to prevent the two from welding together. This anti-weld property of the compounded lubricant is required especially with soft metals and in making deep cuts and working at slow cutting speeds. For harder metals, anti-weld properties are still needed but are associated with extreme pressure additives such as sulfurized or chlorinated fats and waxes which have both cooling and load-bearing properties. They also prevent the formation of too much iron sulfide such as would erode the edge or point of the cutting tool. Hence, a balance between these factors produces the optimum formula for a particular metal or a particular machining operation.

The art shows many types of extreme pressure compounds such as sulfurized fats and esters, chlorinated fats, esters, and waxes, and many other compounds of phosphorous as well as combinations of all these, but very few of the sulfur compounds have anti-weld rather than extreme pressure characteristics. Those that do show anti-weld characteristics are usually present in very small percentages. The total bound sulfur content of most cutting oils is only slightly informative, unless it is first broken down between active and inactive sulfur. Inactive sulfur then should be broken down again between sulfurized fats and the like, which have extreme pressure characteristics and the sulfur naturally in the oil which seems to have neither.

While petroleum may often contain naturally occurring sulfur compounds, these generally lack beneficial properties, may also be odorous and/or corrosive, and are usually removed in the early refining or treatment process. In contrast, various methods have been used to obtain beneficial sulfur by direct introduction of the element (or by injection of sulfur-containing reagents) into fatty oils as well as into (refined) mineral oils. However fatty oils cool the workpiece more than does mineral oil, and hence are less applicable in cutting fluids as they generally lack anti-weld properties and are unable to acquire anti-weld properties without the presence of extreme pressure qualities.

Alternately, sulphur has been incorporated into "additives" such as synthetic polymers, which are then dispersed in the lubricant base to build up a desired concentration of useful sulfur. However, the direct reaction of sulfur with mineral oil has too often yielded a dark colored, malodorous low sulfur content oil from which the sulfur or sulfur-containing precipitate soon separates upon agitation and/or aging. In any event, the amount of useful sulfur permanently introduced by reaction with liquid petroleum lubricant (mineral oil) has been at best no more than about three and a half or four percent, and such procedure has been generally possible only by reacting lubricating fractions of paraffinic base stock with strong reagents at elevated temperature, and in some cases with pressure.

It has now been found however, that by selection of a mildly or incompletely acid-treated, naphthenic-base mineral oil (typically a lubricating oil fraction thereof), a high concentration of useful sulphur (e.g. up to about

2

13% sulfur by weight) can be directly, easily and stably introduced into the petroleum so that the resulting liquid can then be used as a cutting oil per se, or can even be diluted with an equal volume or many volumes of cheaper (depending on the metal to be cut) or local lubricant vehicle and still retain a satisfactory percentage of useful (i.e. active) sulfur having anti-weld properties. Such reaction between the sulfur-containing reagent and the mineral oil can be effected without heating, that is, at ambient room temperature. Although elevated temperature would increase the reaction rate, it is obviously more economical not to heat it.

We have found that a moderate sulfuric acid treatment (i.e. with up to about 10% w. H<sub>2</sub>SO<sub>4</sub>) of naphthene base crude oil (also called asphalt base crude, California or Western crude, Gulf crude, coastal crude, etc.) appears to leave the remaining (dissolved) unsaturated components of the oil more susceptible to a subsequent reaction with certain sulphur compounds so as to form beneficial, solution-stable, sulfur-bearing, organic compounds in the oil. This is in marked contrast to attempted reaction of (the same) crude oil after initial treatment with other extractants such as furfural, "Duosol" (phenol-propane), sulfur dioxide, etc. On the other hand, a more strenuous or complete sulphuric acid extraction of naphthenic petroleum apparently leaves in it only saturated or unreactive components, which, similar to an originally paraffinic crude, subsequently do not react in the present manner to incorporate a high concentration of beneficial and solution-stable sulfur. A viscosity index below about 70 may be taken as an approximate boundary to distinguish the naphthenic base crudes which may be treated by the present invention, as contrasted with the more paraffinic petroleums.

35 Restated: sulphuric acid is commonly used to remove undesirable (especially unsaturated) components from crude oil (by their precipitation, followed by neutralization of the liquid). However, when sulphuric acid treatment is applied to a paraffinic base oil, or is continued to the limit of possible reaction with a naphthenic base oil, it removes all of the unsaturated (and polymerizable) components. Consequently, subsequent introduction of sulfur into the refined petroleum is then possible only to a limited extent and by comparatively strenuous reaction; 40 such practice (when at all effective) has been generally limited to reacting paraffinic type, crude oil following its acid treatment (or its refinement by other means). Now however, by starting with a naphthenic-base crude oil and incompletely acid-treating it, the neutralized liquid is then beneficially reacted with a normally liquid sulfur halide. Such reaction forms in situ, solution-stable, non-malodorous, sulfur-containing organic compounds which are especially beneficial in cutting oil (the entire liquid petroleum reaction-mixture after removal of sludge and volatile components being usable as cutting oil, when it is characterized by other required physical properties, such as viscosity, flash point, etc.). In addition to the reaction compounds subsequently formed in situ by the sulfur halide, the initial "incomplete" sulfuric acid treatment it- 45 self apparently produces some useful compounds which remain in the oil and which possibly may be polymerized by the subsequent reaction with sulfur halide (at least in part). On the other hand, the sulfuric acid removes (as a sludge) various higher molecular weight, reactive 50 compounds which would otherwise later react with the sulfur halide, but would not thereafter permanently remain in solution. Hence the present process increases the yield from the subsequent sulfur halide treatment—in other words, less of the sulfur halide reaction product 55 (as measured by the sulfur content) is lost in the subsequent sludge or precipitate.

By our process, the entire liquid crude oil which possesses any usable lubricating qualities can be sulphurized (generally after removal of tar or heavy residuum, and the topping of gasoline and naphtha portions) and if desired, this overall range which distills from about 300° F. to about 800° F., can be sulfurized following its sulfuric acid treatment, either before or after its fractionation. Or a lubricating oil fraction (e.g. distilling between about 500° F. and about 760° F. and having a viscosity index between about 35 and about -30) such as may be employed in its entirety as a cutting oil may be sulfurized; alternately, under low temperature (refrigerated) operation, a fluid as light as a kerosene fraction can be used as a cutting oil and hence such a volatile portion can be sulfurized with such end use in mind. Such thinner oil has a greater heat transfer value and its comparatively low flash point is of no consequence under frigid operating conditions. On the other hand, a more viscous portion than desired for the ultimate cutting fluid can be sulfurized with the intention of diluting it later with more readily available (or cheaper) diluent—which need not be mineral oil—since a sulphur concentration as high as the obtainable 13% w. is not needed in many cutting liquids. Likewise, the sulfurized fraction can be diluted with less viscous fluid which in addition contains other desired additives such as extreme pressure agents, etc., or the additives can be added to the total vehicle after its dilution. To repeat: the entire usable distillate range of mineral oil can be sulfurized as a unit and subsequently fractionated. Or the liquid petroleum can first be fractionated and (one or more) individual fractions then sulfurized.

"Normally liquid sulfur halide" refers generically to sulfur halides which are liquid at ambient room temperature and atmospheric pressure, such as sulfur-monochloride, sulfur dichloride, sulfur monobromide, thionyl chloride, sulphuryl chloride, or other sulfur halides which are liquid under the conditions under which the reacting petroleum or mineral oil remains liquid. However sulfur monochloride is the most convenient for the present use and the invention will be subsequently exemplified by employment of this reagent. In general, reaction of the sulfur halide with the Western mineral oil evolves some heat and this may be taken as an indication of the petroleum to beneficially utilize the sulfur halide. In general, the potential reactivity is reached with addition of a maximum of about 50% weight  $S_2Cl_2$ . However we prefer to use a smaller quantity and to add this amount in successive fractions over a period of time in order to avoid rapid (temporary) temperature rise and to permit a slower, more stable and complete reaction. Alternately, if it is desired to add the entire quantity of reactant at the beginning, the amount of sulfur monochloride which will remain mixed with the petroleum may be taken as the practical limitation of quantity required. Hence when a permanent layer of the reagent remains separate from the mineral oil after mutual agitation, it may be considered that the petroleum has the required quantity of reactant dispersed therein. When adding the reagent in two or more fractional amounts so as not to effect a gross temperature rise (e.g. no more than about 10° to 20° F.), the reaction is completed in a maximum period of about 12 to 15 hours, or what might roughly be termed "overnight." The odor of sulfur chloride can then no longer be detected upon stirring. Air is blown through the liquid until no odor of hydrogen chloride remains; it may be heated to about 150° F. to about 200° F. to hasten removal of all traces of volatile halide. The small precipitate of insoluble compounds is removed, this is generally on the order of 5% to 30% w. and even this does have the very offensive odor which characterized the in situ sulfurization processes of the prior art.

On the other hand, if the naphthenic crude is reacted first with more than about 10% w. sulfuric acid, this stronger treatment will convert it substantially to a paraf-

finic oil and will remove the compounds which later (by our process) form solution-stable, organic sulfur compounds. While any small amount of concentrated sulfuric acid will have some beneficial effect on the crude oil, 5 treatment with about 0.1% w. may be taken as a practical minimum. About 0.5% w. to about 5% w. has been found quite adequate in most cases. While the present proportions are stated with reference to concentrated sulfuric acid (which is about 95%  $H_2SO_4$  and about 5% water), it will be apparent that since the concentrations described for "acid treatment" are those of the final dilution of mineral oil and sulfuric acid, it is generally irrelevant whether the mixing step is initiated with concentrated 10 or with more dilute sulfuric acid, as long as the final mixture of oil and acid has the designated ratio. Thus, treating petroleum with 1% w. concentrated sulfuric acid, signifies that one percent by weight of the final dilution consists of  $H_2SO_4$ ; it does not mean that a liquid which itself was 1% sulfuric acid was first added to the petroleum. 15 However, since small differences in said concentration are not minutely critical, and in addition since the final result also bears some relation to the time (and temperature) of treatment, it will be apparent that adjustments of the relevant factors will be made by a skilled chemist in applying 20 25 the teaching of the present invention to particular reaction conditions.

In contrast, if the naphthenic crude (in place of sulfuric acid treatment) is refined by any of the various solvent extraction processes (e.g. furfural, sulfur dioxide, propanephenol "Duosol," etc.) a subsequent treatment with sulfur monochloride (with or without heating) will incorporate even less sulfur (e.g. 2.6% w.) than can be incorporated in a paraffinic base oil at elevated temperature, 30 since apparently the extraction process has removed the compounds which would have later incorporated sulfur.

By way of further illustration of our process, a naphthenic base, straight run, Western mineral oil having a distillation range of about 500° F. to about 760° F. and a pour point below -30° F. was agitated with 1% vol. 40 concentrated sulfuric acid at room temperature for 90 min. and then allowed to settle for 4 hours. The acid sludge was separated and the oil neutralized by contact with filtering clay (1% bentonite by wt.); after filtering, the oil had the following analysis:

|    |                                             |         |
|----|---------------------------------------------|---------|
| 45 | Gravity API @ 60° F. -----                  | 20-22.5 |
|    | Viscosity SSU @ 100° F. -----               | 100-110 |
|    | Aniline point, ° F. -----                   | 130-160 |
|    | Neutralization number -----                 | 0.1     |
| 50 | NPA color -----                             | 1-2     |
|    | Pour point, ° F. -----                      | -30     |
|    | Active sulfur (ASTM D-1662-59T) -----       | None    |
|    | Total sulfur (ASTM D-129-58), percent ----- | 0.2     |

55

#### Example 1

To 1 gallon (7.6 lbs.) of the acid-treated oil was added 0.3225 lb. of  $S_2Cl_2$  at room temperature and the mixture agitated by bubbling air therethrough for about 4 hours, then left in the reaction kettle without agitation overnight. The second day another equal portion of  $S_2Cl_2$  added (total of 0.645/7.6 lbs.=8.5% w.), and agitated as before. The end of the reaction was indicated by the absence of sulfur monochloride smell in the effluent vapor. The kettle with its content was then heated to a temperature of 150°-200° F. with air blowing through the body of the oil in order to clear it of all hydrogen chloride. Air continued to be blown through the oil at this temperature about 10 hours until HCl ceased to evolve. (However, there was no appreciable change of the active sulfur content of the oil during this period of heating.) The body of the oil was then left to settle, and the oil was filtered. The resultant product is a dark mahogany color, sulfurized mineral oil, of pleasant odor,

stably homogeneous, and possessing the following characteristics:

|                         |         |
|-------------------------|---------|
| Gravity API @ 60° F.    | 17-17.5 |
| Viscosity SSU @ 100° F. | 130-150 |
| Pour point, ° F.        | -30     |
| Active sulfur, percent  | 5.7     |
| Total sulfur, percent   | 5.9     |
| Yield of oil, percent   | 95      |

*Example 2*

900 gms. of acid treated oil was reacted with 200 gms. of  $S_2Cl_2$ , added in two equal portions, following the procedure of Example 1 above. (Sulfur monochloride 200/900 g.=22% w.) The result was:

|                         |      |
|-------------------------|------|
| Gravity API @ 60° F.    | 15.5 |
| Viscosity SSU @ 100° F. | 200  |
| Active sulfur, percent  | 8.1  |
| Total sulfur, percent   | 8.3  |
| Yield of oil, percent   | 93   |

*Example 3*

800 gms. of acid treated oil reacted with 210 gms. of  $S_2Cl_2$  (=26% w.) added in two equal portions following procedure of Example 1 above. The result was:

|                         |      |
|-------------------------|------|
| Gravity API @ 60° F.    | 13.1 |
| Viscosity SSU @ 100° F. | 245  |
| Active sulfur, percent  | 10   |
| Total sulfur, percent   | 10.2 |
| Pour point, ° F.        | -30  |
| Yield of oil, percent   | 90   |

*Example 4*

700 gms. of the former acid treated oil was reacted with 300 g. (43% w.) of  $S_2Cl_2$  following the procedure of Example 1. The resulting product has the following analysis:

|                         |      |
|-------------------------|------|
| Gravity API @ 60° F.    | 10.6 |
| Viscosity SSU @ 100° F. | 255  |
| Total sulfur, percent   | 13.0 |
| Active sulfur, percent  | 12.8 |
| Yield of oil, percent   | 70   |

*Example 5*

7.6 lbs. of the same cut of naphthenic base oil untreated with sulfuric acid, was reacted with 0.645 lb. of  $S_2Cl_2$  following the procedure in Example 1 above. The resulting product has following analysis:

|                         |      |
|-------------------------|------|
| Gravity API @ 60° F.    | 19.5 |
| Viscosity SSU @ 100° F. | 125  |
| Active sulfur, percent  | 2.0  |
| Total sulfur, percent   | 2.6  |
| Yield of oil, percent   | 75   |

The untreated oil contained 0.6% natural sulfur.

*Example 6*

The procedures outlined in Examples 1, 2 and 3 were followed on a paraffinic base, mineral oil with a similar viscosity as the naphthenic base oil of Examples 1 through 4, as well as examples of higher and lower viscosity. In each instance the yield was an unstable sulfurized oil with a maximum active sulfur of 2.5% w., part of which precipitated out as elemental sulfur within about a week. In addition to the precipitated sulfur, a grayish color sludge was formed which settled down after standing for a week or so.

It will be seen that with increasing concentrations of sulfur monochloride, the viscosity is increased and the API gravity of the final product is lowered and also its yield is decreased, but the amount of incorporated sulfur is increased. Roughly, 50% w. of the sulfur halide is a practical upper limit of concentration, although more could be used, especially if the reaction were effected at lowered temperature and for shorter

periods of time. In general, about 0.5% w. to about 25% w. sulfur halide is preferred; or expressed another way—enough to incorporate up to about 10% w. active sulfur so as to produce an economical concentrate which could be diluted, as needed, with up to four volumes of liquid and still provide a very satisfactory cutting fluid for many purposes, containing approximately 2% w. active sulfur.

The following compositions illustrate some of the uses of our sulphurized mineral oil when mixed with various additives and/or diluents:

*Example 7*

A cutting oil was blended from 23% w. of the product of Example 4, and 77% w. of mineral oil (100 SSU @ 100° F.). The blend contained about 3% w. of active sulfur. When used in threading steel pipe, bright shiny threads with smooth surfaces ensued, and the tool life was up to 40 times longer than when using a commercial mixture of pale oil and sulphurized fatty oil which was recommended for this purpose. In comparison, when using only the recommended commercial product, in addition to the shorter tool life there was produced shredded threads and torn surfaces of the metal which had only a dull finish or appearance.

*Example 8*

A concentrate was formed by mixing the product of Example 4 with an equal volume of sulphurized fat (such as sulphurized sperm oil or sulphurized lard oil). One volume of this concentrate is then blended with two volumes of pale oil of the desired viscosity, at a bulk depot, and distributed to individual users, who then dilute it with from two to ten volumes of pale oil prior to its use on automatic screw machines employed in working various stainless steels. In comparison with a commercial blend of cutting oil recommended for this purpose, our composition produced both extended tool life and smooth finish of the workpiece.

*Example 9*

|                                                                                                           | Percent volume |
|-----------------------------------------------------------------------------------------------------------|----------------|
| Product of Example 4                                                                                      | 20             |
| Miscible oil having extreme pressure properties (such as sulphurized lard oil or other non-petroleum oil) | 10             |
| Refined mineral oil of desired viscosity                                                                  | 70             |

This blend used on a gun drilling machine produced a smoother finish of the workpiece and longer tool life than did a commercial blend of pale oil and sulphurized fatty oil previously used and recommended for this purpose.

*Example 10*

|                            | Percent volume |
|----------------------------|----------------|
| Product of Example 4       | 10             |
| Refined mineral oil SAE 90 | 90             |

Using this blend as a gear oil: after running the motor less than three hours it was impossible to hold one's hand on the gear box due to the overheating produced when the mineral oil alone was used; after adding the 10% of our sulphurized petroleum, it was possible to run the motor indefinitely without overheating.

*Example 11*

Another gear oil, which additionally had extreme pressure characteristics was produced by including 3% vol. lead naphthenate in the preceding formula (the mineral oil then being 87% volume). For drilling and machining metals, other suitable extreme pressure additives include chlorinated hydrocarbons and/or phosphorated hydrocarbons (e.g. tricresyl phosphate). In working carbon steels and stainless steels, as with automatic screw machines, chlorinated additives may be preferred. When used as a long-lasting lubricant, the consistency of grease can be obtained, when desired, by addition of alkali or alkaline-earth soaps (e.g. sodium, lithium or calcium

soaps). In either event, the presence of our sulphurized mineral oil results in longer gear life and smoother performance.

*Example 12*

Another extreme pressure gear oil was compounded of

|                                          | Percent volume |
|------------------------------------------|----------------|
| Product of Example 4                     | 15             |
| Chlorinated paraffin wax                 | 5              |
| Refined mineral oil of desired viscosity | 80             |

In general, a heavy duty petroleum-base gear oil may contain about 10% w. to about 20% w. of our sulphurized mineral oil, about 3% w. to about 20% w. of extreme pressure agents, and the remainder being an inert vehicle consisting essentially of refined mineral oil.

*Example 13*

5% volume of the product of Example 4 was incorporated in a water-soluble mineral oil and the mixture then emulsified with 40 volumes of water. This is sprayed onto the contact face of the iron mold in a glass factory in order to minimize sticking of the glass to the mold. In comparison with such a spray which lacked our sulphurized component, our formula produced a cleaner release operation and resulted in considerable time-saving in cleaning the molds before re-use. Apparently the active sulfur produced by our process, inhibits iron impurities in the glass from adhering to the iron mold. In general, about 1% w. to about 10% w. of our sulphurized petroleum can be mixed with the water-soluble oil, and the mixture is then emulsified with up to as much as about 150 volumes of water to form the sprayable fluid. The aqueous component then volatilizes from the mold surface to leave a thin film of oil.

*Example 14*

In drilling an oil well, the threads of the temporary casing sections became frozen in 40% of the joints when using a commercial pipe thread lubricant recommended for this purpose. After 20% volume of the product of Example 4 was blended into the commercial lubricant, the project was completed without any galling or freezing of joints. In general, such a pipe thread lubricant may contain about 5% w. to about 50% w. of our sulphurized petroleum, about 0.5% w. to about 10% w. of a metallic soap, and the remainder being an inert vehicle consisting essentially of refined mineral oil.

Since such components as extreme pressure agents, mineral soaps used in grease-making, etc., are well known in the lubricant compounding art, they need not be described in detail here. Likewise the various specific proportions recited by way of example in particular formulae are not given by way of limitation but rather as illustrative examples. It is within the competence of a chemist skilled in the art to adopt the teaching and disclosure of our invention to the particular problem at hand; and the breadth of the claimed invention is to be evaluated by reference to the possible substitution of functional equivalents known to the prior art, which may be employed in association with our composition and process.

We claim:

1. The process which comprises reacting a naphthenic-base mineral oil, having a viscosity index below about 70, with about 0.1% w. to about 10% w. of sulfuric acid, such amount of sulfuric acid being less than the maximum amount required to react completely with the oil, removing the sludge formed thereby, neutralizing the oil, reacting it with a normally liquid, sulfur halide, and separating the resulting precipitate and hydrogen halide thereby to leave a stable and homogeneous oil characterized by lack of offensive odor and containing up to 13% w. of active sulfur in oil-soluble organic compounds having anti-weld properties.

2. The process which comprises reacting the lubricating oil fraction of a naphthenic-base mineral oil, with about 0.1% w. to about 10% w. of sulfuric acid, such amount of sulfuric acid being less than the maximum amount required to react completely with the oil, removing the sludge formed thereby, neutralizing the oil, reacting it with a normally liquid, sulfur halide, and separating the resulting precipitate and hydrogen halide therefrom, thereby to leave a stable and homogeneous oil characterized by lack of offensive odor and containing up to about 13% w. of active sulfur in oil-soluble organic compounds which have anti-weld properties, whereby the bulk of said oil containing said soluble compounds is applicable as a cutting oil by itself or upon dilution.
3. The process of the preceding claim 1 wherein said sulfur halide is essentially sulfur monochloride.
4. The process of the preceding claim 2 wherein said lubricating oil fraction has a viscosity index between about 35 and about -30.
5. The process which comprises reacting a naphthenic-base mineral oil, having a viscosity index below about 70, with about 0.1% w. to about 10% w. of sulfuric acid, such amount of sulfuric acid being less than the maximum amount required to react completely with the oil, removing the sludge formed thereby, neutralizing the oil, reacting it with a normally liquid, sulfur halide at ambient room temperature, and separating the resulting precipitate and hydrogen halide therefrom, thereby to leave a stable and homogeneous oil characterized by lack of offensive odor and containing up to about 13% w. of active sulfur in oil-soluble organic compounds which have anti-weld properties.
6. The process of the preceding claim 5 wherein said sulfuric acid is about 0.5% w. to about 5% w. and said sulfur halide is added in fractional amounts during an extended period of time up to about 15 hours, and said reaction is effected principally at ambient room temperature with agitation effected by passage of an air current through the reaction mixture until no odor of sulfur halide or hydrogen halide is evident in the effluent air even upon heating to about 200° F.
7. The process of the preceding claim 6 wherein said sulfur halide is essentially about 0.5% w. to about 25% w. of sulfur monochloride.
8. The process which comprises reacting the lubricating oil fraction of a naphthenic-base mineral oil, with about 0.5% w. to about 5% w. of sulfuric acid, such amount of sulfuric acid being less than the maximum amount required to react completely with the oil, removing the sludge formed thereby, neutralizing the oil, reacting it at ambient room temperature with up to about 50% w. of sulfur monochloride, and separating the resulting precipitate and all volatile chlorides therefrom, thereby to leave a stable and homogeneous cutting oil or additive therefor, characterized by lack of offensive odor and containing up to about 13% w. of active sulfur in oil-soluble organic compounds which have anti-weld properties.
9. A mineral oil base, cutting fluid containing homogeneously and stably dispersed therein, an anti-weld quantity of the organic, oil-soluble reaction product formed between a normally liquid, sulfur halide and a naphthenic-base mineral oil having a viscosity index below about 70; said reaction product being formed by treating said mineral oil with about 0.1% w. to about 10% w. of sulfuric acid, such amount of sulfuric acid being less than the maximum amount required to react completely with the oil, removing the sludge formed thereby with the sulfuric acid and neutralizing the remaining oil, and then reacting the neutralized oil with said normally liquid sulfur halide and separating the resulting precipitate and hydrogen halide therefrom, thereby leaving an organic, oil-soluble reaction product containing up to about 13% w. active sulfur and having consequent anti-weld properties, said reaction product remaining dissolved in the mineral oil in

which it was formed, which oil forms the bulk of said cutting fluid.

10. The cutting fluid of the preceding claim 9 wherein said normally liquid, sulfur halide consists essentially of sulfur monochloride, and said reaction product contains from about 4% w. up to about 13% w. of active sulfur based on the weight of said naphthenic base mineral oil.

11. The cutting fluid of the preceding claim 10 wherein said reaction product is formed essentially at ambient room temperature.

12. The cutting fluid of the preceding claim 9 wherein said naphthenic-base mineral oil, prior to said sulfuric acid treatment, consists essentially of a lubricating oil fraction of said mineral oil.

13. A fluid composition having lubricant and anti-weld properties and characterized by a beneficial quantity of the reacted mineral oil of claim 9 generally uniformly dispersed in a lubricant vehicle.

14. The cutting fluid of the preceding claim 9 wherein said naphthenic-base mineral oil, prior to said sulfuric acid treatment, consists essentially of a lubricating oil fraction of said mineral oil, and said normally liquid, sulfur halide consists essentially of sulfur monochloride which is reacted with the sulfuric-acid-treated-oil essentially at ambient room temperature.

15. The composition of the preceding claim 13 wherein said vehicle includes water which is emulsified with said fluid whereby said composition is adapted to be sprayed onto a metallic mold and thus to serve as a mold release agent.

16. The composition of the preceding claim 13 wherein said vehicle includes an added amount of an extreme pressure agent.

17. The composition of the preceding claim 13 wherein said vehicle includes an added amount of miscible, sulfurized, non-petroleum oil having extreme pressure properties.

18. The composition of the preceding claim 13 wherein said vehicle comprises refined mineral oil and a grease-forming quantity of metallic soap.

19. A pipe thread lubricant comprising about 5% w. to about 50% w. of the fluid of claim 10, about 0.5% w. to about 10% w. of a metallic soap, and the remainder being an inert vehicle consisting essentially of refined mineral oil.

20. A petroleum-base gear oil comprising about 10% w. to about 20% w. of the fluid of claim 10, about 3% w. to about 20% w. of extreme pressure agent, and the remainder being an inert vehicle consisting essentially of refined mineral oil.

21. A sprayable mold-release fluid consisting essentially of a mixture of about 1% w. to about 10% w. of the fluid of claim 10 and about 90% w. to about 99% w. of refined mineral oil, which mixture is emulsified with from about 40 to about 150 volumes of water.

#### References Cited by the Examiner

##### UNITED STATES PATENTS

|           |         |               |       |          |
|-----------|---------|---------------|-------|----------|
| 1,824,523 | 9/1931  | Adams         | ----- | 252—45   |
| 2,112,677 | 3/1938  | Muskat        | ----- | 252—45   |
| 2,142,916 | 1/1939  | Parkhurst     | ----- | 252—45   |
| 2,246,282 | 6/1941  | Zimmer et al. | ----- | 252—45   |
| 2,303,853 | 12/1942 | Lutz et al.   | ----- | 252—45   |
| 2,378,803 | 6/1945  | Smith         | ----- | 260—139  |
| 2,380,072 | 7/1945  | Reid          | ----- | 260—139  |
| 2,578,865 | 12/1951 | Veatch et al. | ----- | 252—49.5 |

##### OTHER REFERENCES

Manufacture and Application of Lubricating Greases, C. J. Boner, Reinhold Publishing Corp., 1954, pp. 152—157.

DANIEL E. WYMAN, Primary Examiner.

L. G. XIARHOS, Assistant Examiner.